

April 21, 1925.

1,534,861

H. C. MARTIN

ABRASIVE DISK

Original Filed Jan. 25, 1922

*Fig. 1.*



*Fig. 2.*



*Fig. 3.*



INVENTOR  
Harry C. Martin  
By Raymond Robbins, Attorney  
His Atty

## UNITED STATES PATENT OFFICE.

HARRY C. MARTIN, OF NIAGARA FALLS, NEW YORK, ASSIGNOR TO THE CARBORUNDUM COMPANY, OF NIAGARA FALLS, NEW YORK, A CORPORATION OF PENNSYLVANIA.

## ABRASIVE DISK.

Original application filed January 25, 1922, Serial No. 531,554. Divided and this application filed January 30, 1924. Serial No. 689,431.

*To all whom it may concern:*

Be it known that I, HARRY C. MARTIN, a citizen of the Dominion of Canada, residing at Niagara Falls, Niagara County, New York, have invented a new and useful Improvement in Abrasive Disks, of which the following is a full, clear, and exact description, reference being had to the accompanying drawings, forming part of this specification, in which.

Figures 1 and 2 are sectional views of mold devices and illustrating steps in the manufacture of the abrasive disks; and

Figure 3 is a perspective view of a finished disk embodying my invention.

This application is a division of my pending application, Serial No. 531,554, filed January 25, 1922.

My invention relates to an improvement 20 in abrasive disks, these disks being of the character used on machines known as "disk grinders," for grinding flat surfaces on metals and other materials. Such disks usually consists of a paper or cloth backing or body 25 coated with a thin layer of abrasive by means of glue after the ordinary manner of sand paper and emery cloth. Their use is limited by the fact that the coating is relatively thin, and they do not possess very much durability when called upon to do heavy work. Their usefulness is also to a large degree conditioned upon the degree of porosity of the abrasive, the porosity being the measure of the free cutting properties of 35 the material. This is due to the fact that the degree of porosity controls freedom from glazing in use; or in other words, the free cutting properties of the disk depend upon the extent to which the material ground off 40 is kept from lodging in the pores of the cutting surfaces.

I have discovered that a very efficient abrasive disk can be made by building up an abrasive body consisting of abrasive grains 45 bonded together by a resinous cement, preferably of shellac, upon a backing of cloth or paper.

In the practice of my invention, for example in the making of a shellac disk, I employ a shallow circular mold consisting of an iron bottom plate 2 and an iron ring 3 of the proper diameter required for the disk. In this mold, I place a disk 4 of cloth or paper and spread over this a thin layer from three-sixteenths of an inch to three-fourths

of an inch thick of abrasive grains mixed with powdered shellac, preferably in approximately the proportions by weight of ninety-two parts abrasive grains and eight parts powdered shellac, although the exact 60 proportions may be varied somewhat to meet the characteristics desired in the particular disk being manufactured. The shellac should, in general, not exceed nine or ten per cent of the mix, as shellac in excess of 65 this makes the disk too hard and dense.

The mold with its contents is then placed in the melting oven and brought up to a temperature sufficient to bring the shellac to a molten or plastic condition. The mold is 70 then taken from the oven and a circular iron plunger, such as illustrated at 5 in Figure 2, is inserted in the ring 3 upon the abrasive material, and the latter is subjected to pressure of three hundred to five hundred pounds, 75 per square inch, which compresses and agglomerates it. Increasing the proportion of shellac and the pressure increases hardness and decreases the porosity of the disk. I have used in practice from eight to ten percent of shellac and have varied the agglomerating pressure from three hundred to five hundred pounds, per square inch, to meet the variations in hardness that are required. The disk is then removed from the mold and 80 allowed to cool, after which it is baked in an oven at a temperature, preferably of from two hundred and ninety to three hundred degrees Fahrenheit.

If the baking temperature does not exceed 90 three hundred degrees Fahrenheit, the paper or cloth backing is not destroyed and is available for the purpose of forming an intermediate layer between the disk and the plate upon which the disk is fastened, when 95 put into actual use.

As a modification of the above described method, I may, however, bake at a temperature of three hundred and fifty degrees Fahrenheit. This temperature destroys the 100 backing, but toughens and improves the abrasive. I then take a fresh piece of backing material and shellac it on to the abrasive disk by means of freshly melted shellac. In this manner, I obtain a combination of the 105 shellac body and backing in as good a working condition as if the backing was originally incorporated with the shellac body.

It will be understood that the backing 110 serves two functions, viz., it acts as a means

of holding and carrying the disk body in its first melted condition and to strengthen the same until it is transferred to the baking operation, where it is toughened until it no longer needs such reinforcement. The second function is to form an intermediate layer between the disk and plate, as above stated. Both these functions may be performed by the modification above described, as well as by the first described method.

I have found that disks made in accordance with my invention, using ordinary artificial aluminous abrasives in grits from No. 16 to No. 36, will weigh from 1.9 to 2.3 grams per cubic centimeter. The apparent density of two grams per cubic centimeter gives a very good cutting efficiency, and the disk does not glaze up with the material being ground, but maintains a very good cutting surface. With apparent densities of from 1.9 to 2.3 grams per cubic centimeter, the equivalent porosity varies from 47 to 36 percent; and it is important that the porosity should not be less than 36 percent, 20 in order to give the free cutting properties above described.

An ordinary shellac bound grinding wheel made up according to the methods heretofore in use with grits of these sizes and 30 grades, has an apparent density of from 2.4 to 2.6 grams per cubic centimeter, and if used in the same cutting operation would very quickly glaze and show very poor cutting efficiency.

In making such grinding wheels the amount of shellac and the agglomerating pressure greatly exceed that employed in making my grinding disks.

In addition to the increased porosity, the disks made in accordance with my invention have a uniform texture throughout so that they will remain efficient during their life. They also possess the advantage that they do not crack or chip at the edges. They may be used either wet or dry, which is not true of a glued disk. The disks may be made of any desired grade of hardness to suit the particular work in which they are to be used.

While the disks have sufficient porosity to 50 prevent glazing, they have sufficient strength and density to stand up under hard usage, and have a durability and cutting efficiency much greater than disks made of abrasive material not compressed. The disks may also be built up to any thickness desired,

which is not practical in making disks in which abrasive is sprinkled on to the adhesive. The shellac gives a good tensile bond, and the disks are capable of operating more safely and under higher peripheral speeds than disks having weaker bonding materials, such for example, as magnesia cement. The abrasive composition of the disks is considerably more porous, and hence, structurally not as strong as the 65 more dense shellac bound abrasive wheels containing a greater percentage of shellac and made with a higher agglomerating pressure. However, the cloth backing of my disks supplies an added tensile strength, so that the composite disks are capable of safely operating at the high peripheral speeds now used in disk grinding. The disks, therefore, combine high enough porosity to prevent glazing, sufficient thickness, 70 strength of bond and density to have great durability, and the necessary tensile strength for high speed grinding machinery.

While I have described in detail the preferred embodiment of my abrasive disk and its process of manufacture, it is to be understood that the invention is not limited to all of the described details, but may be otherwise embodied within the scope of the 75 following claims.

I claim:

1. An abrasive disk comprising a backing of flexible material and an abrading portion built up of abrasive grains and a resinous bonding material and having a porosity of 90 not less than 36%, substantially as described.
2. An abrasive disk comprising a backing of flexible material and an abrading portion built up of abrasive grains and a resinous bonding material and having a porosity in excess of 40%, substantially as described.
3. An abrasive disk comprising a flexible backing and an abrading portion formed of a compressed mixture of abrasive grains and with not over 10% of shellac as a bonding material, substantially as described.
4. An abrasive disk comprising a flexible backing and an abrading portion formed of a compressed mixture of abrasive grains and with 8 to 9% of shellac as a bonding material, substantially as described.

In testimony whereof I have hereunto set my hand.

HARRY C. MARTIN.